

# United States Patent Office

2,748,069

Patented May 29, 1956

1

2,748,069

## TRIVALENT CHROMIUM PLATING SOLUTION

Jean Jacques Georges Icxi, Paris, France

No Drawing. Application July 27, 1953,  
Serial No. 370,640

Claims priority, application France March 20, 1948

13 Claims. (Cl. 204—51)

This invention is concerned with an electroplating solution of chromium, which allows obtaining very quickly a chromium coating of very good physical and mechanical properties.

The present application is a continuation-in-part of my co-pending application Serial Number 82,264 filed March 18, 1949, now abandoned.

More than a hundred patents have described electroplating solutions in which chromium is present in the form of chromic acid or salts of this acid, that it to say in the hexavalent state. These solutions give rise to a number of difficulties; many attempts have been made to overcome them by adding to these solutions small amounts of various organic and mineral compounds. But, whatever be the nature of such additions, their low proportions do not change the nature of these solutions which remain solutions of hexavalent chromium, as is clear to those skilled in the art. All the solutions so constituted have the known inconveniences of hexavalent chromium solutions, among others, the necessity that the surface to be plated be perfectly clean, and the necessity to operate at or about room temperature and with low current densities, generally no higher than 12 to 15 amperes per square decimeter.

As it will appear from this specification, the solutions according to the invention do not exhibit the above noted drawbacks.

Plating solutions in which chromium is present in the hexavalent state are poisonous, are corrosive, and liberate toxic gaseous products during electrolysis. These poisonous characteristics do not exist in the solutions according to the present invention.

The electro-plating solution according to the present invention is characterized in that it contains only at least one salt formed by a complex anion constituted by trivalent chromium and at least one organic acid and by a cation which is an amine base.

The anion of such complex salt is thus constituted by an atom of trivalent chromium associated with six radicals of a monocarboxylic organic acid, or three radicals of a di-carboxylic organic acid, these acid radicals being identical or different. This anion is thus trivalent, as the chromium is itself trivalent, and is consequently neutralized by a cation having three radicals of an amine base, these radicals being identical or different. In general, the organic acid has less than six atoms of carbon and the amine has at most six atoms of carbon.

It is not necessary to employ a single organic acid or a single amine base, to constitute a solution according to the present invention. According to the present invention, it is possible to employ a chromium salt of one organic acid and an amine base salt of another organic acid. It is also possible to employ a mixture of different salts of different amine bases.

According to Werner's classification, described in the book "Introduction à la chimie des complexes" by Georges Urbain et Séchéchal, edited by Herman et fils, Paris 1913,

2

the salts as employed according to the present invention are represented by the general formula

[Cr (acid radicals)] (amine)

5 where "acid radicals" designate the radicals of at least one organic acid, having each less than six atoms of carbon and the number of which radicals being such that the sum of their valences is equal to six, and where "amine" designates the ammonium radical or the radicals of at least one 10 amine having at most six atoms of carbon, the number of said amine basic radicals being such that the sum of their valences is equal to three. Ammonium is considered as an amine radical.

As these salts are intended to be used in solution, the 15 acids and amines which are suitable are those which produce a soluble complex salt, that is to say acids whose number of carbon atoms is lower than six and amines whose number of carbon atoms is lower than six.

The expression "complex salt" is employed in the present specification and claims to denote a salt of the kind indicated hereinbefore, in the molecule of which the organic acid radicals are identical, and the amine radicals are also identical. I make use of the terms "mixed complex salt" to designate a salt in the same molecule of 25 which are included different carboxylic organic acid radicals and/or amine radicals.

According to the present invention, in general, using a trivalent anion of chromium, an amount of chromium hydroxide corresponding to a molecule of chromium is 30 dissolved in an amount of

$\frac{6}{n}$

molecules of at least one carboxylic organic acid,  $n$  being 35 the number of carboxylic groups in the acid radical.

Many actual tests under operating conditions made on an industrial scale have shown that such electro-plating solution according to the present invention can be employed at temperatures as high as the boiling point of the 40 plating solution and with current densities higher than 300 amperes per square decimeter.

In usual practice, the current density is about 200 amperes per square decimeter.

The process according to the present invention is satisfactory for plating small work pieces under very high current densities.

In these plating solutions, all according to the present invention, chromium is present only in a complex anion. During electrolysis, the object to be plated being the 50 cathode, there is first obtained the well known phenomenon according to which the complex anion is transferred to the anode and the amine radical to the cathode, which is always surrounded by an alkaline medium; as the complex anion cannot remain in this form, it is split 55 down into a chromium ion and an acid ion which remains near the anode, the chromium being transported towards and plated on the cathode. As the latter is always alkaline, there is no need that the object to be plated be perfectly clean or scoured.

60 As the chromium must be completely present only as a complex ion, the proportions of the components used to prepare the solutions must be about those theoretically in accordance with the formula of the salt to be prepared. It is not necessary to insist rigorously upon that condition, 65 which is well known to those skilled in the chemistry of chromium complexes.

The plating solutions according to the present invention have a pH of about 7, and the chromium is in the form of a complex of the kind indicated above. This 70 condition is fulfilled when there occurs no formation of an insoluble chromium precipitate following a com-

plete alkalization of the solution. Should such a precipitate be formed, it will be sufficient to add a further amount of the salt of the amine base, or of the acid.

A solution according to the present invention may be obtained by directly dissolving in a convenient amount of water a complex salt of chromium of the kind above specified, with the addition of a salt of an amine base if necessary.

This solution according to the present invention may also be obtained indirectly. According to a first embodiment, I prepare a solution of an organic salt of trivalent chromium to which I add a solution of an organic salt of the selected amine base. I can also dissolve the amine base in the total necessary amount of organic acid, and then I dissolve in this solution the proper amount of hydroxide or basic carbonate of chromium.

I can also start from a solution of a mineral salt of chromium such as the violet sulphate of chromium, to which I add the proper amounts of an organic salt of the selected amine and of an organic acid, and I treat the resulting solution by an amount of hydrated baryta corresponding to the amount of sulphuric ion of the sulphate. Barium sulphate being insoluble, the solution is free from mineral compounds.

The alkalinity or acidity of the raw solution obtained according to one or the other of the above mentioned processes may be corrected by a convenient addition of organic acid or amine base so as to bring the pH of the solution to a pH value of about 7.

According to a particular aspect of the present invention, platings may be obtained which are constituted by chromium alloys. To this end, I add to the solution of a complex salt of trivalent chromium, a soluble salt of a metal such as iron, nickel, cobalt, etc., which is compatible therewith, as shown by a preliminary test; the electroplatings of the other metal and of chromium are effected simultaneously.

Moreover, the chromium coatings obtained from a solution according to the present invention are more or less "carburized," that is to say contain a part of the chromium in the form of chromium carbide. This characteristic is particularly outstanding when the solution contains a formic complex of trivalent chromium and/or when the anode is constituted by a graphite piece.

In using solutions according to the present invention in chromium plating, the usual apparatus and operating conditions are employed, and the concentration during electrolysis, are substantially normal, but the allowable current densities and temperature of the electrolyte are much greater than permissible in the prior art.

The solutions according to the present invention are particularly useful when they are employed in the so-called "spot plating method" in which an absorbent mass connected to the positive pole of a source of electric current is soaked in the solution and is applied to the object to be plated which is connected to the negative pole of the source of current. This method can be applied with apparatus of the kind described in my co-pending application Serial No. 321,327.

The following examples, which are purely illustrative and should not be construed in limitative sense, will illustrate how a solution according to the present invention can be obtained.

#### Example 1

For a final volume of 1000 cm.<sup>3</sup>, 700 grams of the chromium oxalate known as ammonium Gregory salt, having the formula



are dissolved in water, with the aid of heat. The chromium is present as trivalent chromium.

Gregory salt is described in Zeitschrift f. Anorganische Chemie, v. 11, p. 209 (1896) and v. 21, p. 8 (1899), and in Pascal, Traité de Chimie Minérale, vol. 10, pages

1074-1075, Paris 1933, and in an article by Bussy, Liebigs Annalen der Chemie, vol. 29, page 312 (1839).

The solution thus obtained, electrolyzed under 150 amperes per square decimeter with platinum anode, yields a chromium coating of a light blue color and which exhibits very good physical and mechanical properties.

#### Example 2

The two following industrial solutions are mixed in the proportion of:

6 volumes of a solution of chromium formate containing 200 grams per liter of the anhydrous salt, the chromium being present as trivalent chromium, and 4 volumes of a solution of ammonium formate at 16° Baumé, containing 610 grams per liter of this ammonium formate salt.

After digestion for an hour at 80° C. the resulting solution is brought to neutrality with pH of 7, in the cold. The salt so obtained has the following formula:



its solution yields white coatings, both with the tank and the spot methods.

#### Example 3

In the hot way, 100 grams of chromic acid titrating more than 90% of pure acid are reduced by adding 370 grams of formic acid of 90% by weight, partly neutralized by 200 grams of ammonia water of 26% by weight of NH<sub>3</sub>. When the reduction is complete, the solution is brought to neutrality by adding a sufficient amount of ammonia water, and its volume is adjusted to a value of 600 cm.<sup>3</sup>. There is so obtained the same complex salt as in Example 2.

This solution, electrolyzed under 250 amperes per square decimeter with graphite anode, yields chromium coatings of very good properties with a surprising rapidity.

In this example, the chromium is present during electrolysis as trivalent chromium. The chromic acid is reduced by the formic acid to yield chromium formate, according to the reaction:



This reduction entirely eliminates all hexavalent chromium which was originally present in this example in the chromic acid, so that there is present during electrolysis only trivalent chromium as chromium formate, and an excess of formic acid which is then neutralized by ammonia.

#### Example 4

Moist precipitated hydroxide of chromium, in an amount corresponding to 76 grams of (trivalent) Cr<sub>2</sub>O<sub>3</sub>, is dissolved in the hot way in a sufficient amount of water by a mixture of 200 grams of crystallized oxalic acid and 175 grams of succinic acid. This latter mixture corresponds to an amount of

molecules of organic acid, where n is the valence of the organic acid that is the number of carboxylic groups in the acid radicals.

The solution is partly neutralized by 60 grams of ammonia of 26% by weight of NH<sub>3</sub>. After it has dissolved, there are added 35 grams of hydrazine of 50% by weight and approximately from 60 to 70 grams of ammonia of 26% to attain neutrality (about pH 7), and the volume of the solution is brought to 1000 cm.<sup>3</sup> with water.

The complex salt so obtained has the following formula:



5

## Example 5

To 500 cm.<sup>3</sup> of an industrial solution of green (trivalent) chromium sulphate at approximately 30° Baumé, containing 300 grams of the anhydrous salt for one liter, there are added at 70° C.: 500 cm.<sup>3</sup> of a solution of ammonium formate at 16° Baumé, containing 610 grams per liter of this salt, and 120 grams of formic acid of 90% by weight.

This solution is then treated by 350 grams of hydrated baryta, heated, and the precipitate of barium sulphate thus formed is filtered away. The solution so obtained is brought to pH of about 7, and 100 cm.<sup>3</sup> of methyl alcohol are added thereto.

This solution, which contains a complex salt having the following formula:



yields white platings, even in a tank, under strong density of current.

## Example 6

An amount of moist chromium hydroxide corresponding to 100 grams of (trivalent) Cr<sub>2</sub>O<sub>3</sub> is dissolved in the cold in 200 cm.<sup>3</sup> of water by means of 200 grams of 90% by weight formic acid which has less than six atoms of carbon. The resulting solution is rapidly mixed with a solution of formate of methylamine, having a pH of about 7, which is obtained by the neutralization of 400 grams of an aqueous solution of 33% by weight methylamine by means of about 200 grams of 90% by weight formic acid. The formic acid is an organic acid having less than six atoms of carbon, and the methylamine is an amine having at most six atoms of carbon.

The solution is maintained during 15 to 30 minutes at a temperature of 70–80° C. and is then alkalinized (pH=7.5) by the addition of a small calculated amount of the solution of the amine. The resulting solution, which contains a complex salt having the following formula:



is brought to 1000 cm.<sup>3</sup> and yields very good platings by electrolysis at temperature higher than 40° C.

## Example 7

An amount of moist chromium hydroxide corresponding to 100 grams of Cr<sub>2</sub>O<sub>3</sub> is dissolved in the cold in 200 cm.<sup>3</sup> of water by means of 200 grams of 90% formic acid. The resulting solution is rapidly mixed with a solution of formate of dimethylamine (CH<sub>3</sub>)<sub>2</sub>NH, obtained by the neutralization of 850 grams of an aqueous solution of dimethylamine of 25% by weight by means of about 200 grams of 90% formic acid.

The solution thus obtained is then treated as indicated in Example 6. It contains a complex salt having the following formula:



## Example 8

To 6 volumes of an industrial solution of (trivalent) chromium acetate at 20° Baumé, containing 250 grams per liter of the anhydrous salt, there are added 7 volumes of a solution of ammonium acetate at 11° Baumé containing 450 grams of this salt per liter.

The resulting solution is maintained during six hours at a temperature of 70° C., then cooled and brought to a pH of about 7 by a careful addition of ammonia water.

The complex salt so obtained has the following formula:



6

## Example 9

500 grams of Gregory's salt of potassium as identified in Example 1 above, having the following formula:



are dissolved at 80–90° C. in 500 cm.<sup>3</sup> of water. When this salt is dissolved, there are added 300 grams of sulphate of hydroxylamine SO<sub>4</sub>(NH<sub>2</sub>OH)<sub>2</sub> and the mixture is agitated for half an hour. Then the temperature is brought to 60–80° C. and this temperature and the agitation is maintained for one hour. The separated potassium sulphate is filtered off hot. The chromium is present as trivalent chromium.

The solution is then concentrated and again submitted to crystallization, and the separation of the potassium sulphate is achieved through an addition of 10% by volume of ethyl alcohol. The solution so obtained is brought to 1000 cm.<sup>3</sup> with water. There is obtained a solution of the oxalic chromium complex salt of hydroxylamine, having the following formula:



## Example 10

25 In the embodiment described in Example 2, formate of hydroxylamine may be partly substituted for ammonium formate and there are obtained the following compounds:



30 or



according to the respective proportions of hydroxylamine and ammonium formate. These proportions can be easily determined from the above given formulae, as is well known by those skilled in the art. The chromium is present as trivalent chromium.

All these salts comprising an hydroxylamine ion yield very bright chromium platings.

## Example 11

40 750 grams of tertiary amylamine (dimethyl-ethyl carbylamine) having the formula:



45 are added to 600 cc. of water and are neutralized by means of 250 grams of 90% formic acid. The solution is heated to 80° C. and mixed with 500 cc. of a solution of violet sulphate of chromium (trivalent) at about 30° Baumé, containing 300 grams per liter of the anhydrous salt.

50 To the solution thus obtained, there are added 500 grams of barium formate and the mixture is maintained 12 hours at 80° C. under agitation. During that time, the pH of the solution is kept between pH 6 and pH 7. Then, the precipitate of barium sulphate thus formed is filtered away. The solution is now cooled, its pH is adjusted to pH 6.5 by an addition of formic acid or of tertiary amylamine, and its volume is brought to 2000 cc. There is obtained a complex salt having the formula:



## Example 12

A complex salt having the following formula:



70 is obtained if the 750 grams of dimethyl-ethyl-carbylamine of Example 11 is replaced by 300 grams of allylamine (2-propenylamine) having the formula



the treatment being otherwise the same, except that the volume of the resulting solution is brought to 1500 cc. The chromium is present as trivalent chromium.

*Example 13*

In the process according to Example 11, use is made of 275 grams of technical diethyl-triamine, having the formula:



instead of 750 grams of dimethyl-ethyl-carbylamine. The treatment is the same in other respects except that the solution is brought to 1250 cc. and the pH adjusted to a value of 7. The complex salt obtained has the formula:



The chromium is present as trivalent chromium.

*Example 14*

An amount of moist chromium hydroxide corresponding to 100 grams of  $\text{Cr}_2\text{O}_3$  (trivalent) is dissolved in a hot solution of 270 grams of maleic acid, having the formula:



in 200 cc. of water.

To this solution is added, at 70° C., a solution of neutral ammonium maleate, obtained by dissolving 270 grams of maleic acid in 250 cc. of water and neutralizing by means of 250 cc. of a solution of ammonia of 34% by volume.

The resulting solution is filtered, brought to a volume of 1000 cc. and its pH is adjusted to a value of 7 to 7.5 by a careful addition of ammonia water. There is obtained a complex salt having the following formula:



*Example 15*

The same operations are made as in Example 14 but the two amounts of 270 grams of maleic acid are replaced by two successive amounts of 325 grams of propionic acid:  $\text{CH}_3\text{---CH}_2\text{---CO}_2\text{H}$ . The following complex salt is obtained:



*Example 16*

If two successive amounts of 300 grams of glutaric acid:  $\text{CO}_2\text{H---CH}_2\text{---CO}_2\text{H}$  are substituted for the 270 grams of maleic acid of Example 14, the following complex salt is obtained:



*Example 17*

The two following industrial solutions are mixed in the proportions of 6 volumes of solution of (trivalent) chromium acetate of 20° Baumé containing 250 grams per liter of the anhydrous salt and 4 volumes of solution of ammonium formate of 16° Baumé containing 610 grams per liter of this salt. The mixture is maintained during one hour at 80° C. and is then brought to a pH of 7 by a careful addition of ammonia water. The solution yields very good white coatings. The complex salt obtained has the formula:



In this example there are present two different organic acids having each less than six atoms of carbon, the number of carboxylic groups present in said acid being such that the sum is equal to six, and there are present radicals of an amine having at most six atoms of carbon,

the number of basic radicals being such that their sum is equal to three.

In all of the foregoing examples, in no case does the organic radical employed have more than five carbon atoms, nor does the amine employed have more than six carbon atoms.

The chromium plating solutions which have been here described can be used for special electrolyzing methods, such as those known as "spot or plugging or pencilling galvanoplasty." These solutions can be electrolyzed using high current densities such as 200 to 300 amperes per square decimeter, and at temperatures as high as the boiling temperature of the solution itself. This is an important advantage of the plating solution here described.

Tests have been made for the purposes here in view of many mineral compositions of chromium. Under the conditions required for the purposes here in view, these compositions have either not given any deposits at all, or, particularly in the case of compositions having complex anions of chromium and mineral acids, have given black deposits, more or less pulvurulent, and entirely useless for industrial purposes. Only the compositions described in this present application have been found to produce the types of satisfactory deposits and the results which have been set forth in this application.

It has been found that any addition of mineral compositions to the solutions which have been here described, have the effect of deteriorating the deposits obtained, the deterioration becoming more serious as the proportions of such additional mineral compositions added becomes larger. If to chromium plating solutions of the prior art, such as those containing chromic acid and an ammonium organic salt, there is added simply a more or less large quantity of organic acid or amine, these additions cannot change the nature of the solution, and cannot attain the results here set forth, which require a complete change of the nature of the solution. Particularly these additions do not eliminate the mineral components of the solutions of the prior art, which components are undesirable as above explained.

The chromium plating solutions which have been here described alone present the following advantages which are not to be found in the solutions known to the prior art.

a. Deposits can be obtained with current densities as high as 300 amperes per square decimeter.

b. Deposits can be obtained at temperatures going up to the boiling temperature of the solution.

c. Under the conditions specified in paragraphs a and b above, the solutions according to the present invention are the only ones to give thick deposits, extremely hard and brilliant, and this within a very short time.

d. All heretofore known plating solutions, especially of hexavalent chromium, are toxic and possess necroscopic properties, which is particularly dangerous. In chromium plating solutions according to the present invention, these toxic and necroscopic properties are entirely absent.

e. Since the results above enumerated under a, b, c, d, are obtained only when the chromium is present in the state of the complex as described in the present specification, the proportions indicated in the examples as given, for the components present in the solution, are critical and of great importance, since the formation of the intended complexes depends on the employment of these specified proportions.

The results which have been described as having been attained with the present invention, are all new results, which have not been attained with the chromium plating solutions of the prior art, and the solutions according to the present invention therefore constitute important advances in the art.

What I claim is:

1. A chromium electroplating bath of a pH of about 7 consisting of an aqueous solution of at least one com-

plex salt of trivalent chromium corresponding to the formula:



5

wherein "acid" designates at least one organic carboxylic acid radical having less than six carbon atoms, "n" designates the number of carboxylic groups in said acid radical, and "amine" designates at least one radical selected from the group consisting of amine and ammonium radicals, said amine radical having at most six carbon atoms.

2. A method of electrodepositing chromium upon a cathodic base which comprises passing an electrolytic current from an anode to said cathodic base through a chromium electroplating bath of a pH of about 7 consisting of an aqueous solution of at least one complex salt of trivalent chromium corresponding to the formula:



15

wherein "acid" designates at least one organic carboxylic acid radical having less than six carbon atoms, "n" designates the number of carboxylic groups in said acid radical, and "amine" designates at least one radical selected from the group consisting of amine and ammonium radicals, said amine radical having at most six carbon atoms.

3. A method of electrodepositing chromium upon a cathodic base which comprises passing an electrolytic current from an anode to said cathodic base through a chromium electroplating bath of a pH of about 7 consisting of an aqueous solution of at least one complex salt of trivalent chromium corresponding to the formula:



25

wherein "acid" designates at least one organic carboxylic acid radical having less than six carbon atoms, "n" designates the number of carboxylic groups in said acid radical, and "amine" designates at least one radical selected from the group consisting of amine and ammonium radicals, said amine radical having at most six carbon atoms, the current density on said anode and cathode exceeding one hundred and fifty amperes per square decimeter.

4. A chromium electroplating bath of a pH of about 7 consisting of an aqueous solution of a complex salt of trivalent chromium corresponding to the formula:



45

5. A chromium electroplating bath of a pH of about 7 consisting of an aqueous solution of a complex salt of trivalent chromium corresponding to the formula:



6. A chromium electroplating bath of a pH of about 7 consisting of an aqueous solution of a complex salt of trivalent chromium corresponding to the formula:



60

7. A chromium electroplating bath of a pH of about

7 consisting of an aqueous solution of a complex salt of trivalent chromium corresponding to the formula:



8. A chromium electroplating bath of a pH of about 7 consisting of an aqueous solution of a complex salt of trivalent chromium corresponding to the formula:



9. A method of electrodepositing chromium upon a cathodic base which comprises passing an electrolytic current from an anode to said cathodic base through a chromium electroplating bath of a pH of about 7 consisting of an aqueous solution of a complex salt of trivalent chromium corresponding to the formula:



20 10. A method of electrodepositing chromium upon a cathodic base which comprises passing an electrolytic current from an anode to said cathodic base through a chromium electroplating bath of a pH of about 7 consisting of an aqueous solution of a complex salt of trivalent chromium corresponding to the formula:



11. A method of electrodepositing chromium upon a cathodic base which comprises passing an electrolytic current from an anode to said cathodic base through a chromium electroplating bath of a pH of about 7 consisting of an aqueous solution of a complex salt of trivalent chromium corresponding to the formula:



30 12. A method of electrodepositing chromium upon a cathodic base which comprises passing an electrolytic current from an anode to said cathodic base through a chromium electroplating bath of a pH of about 7 consisting of an aqueous solution of a complex salt of trivalent chromium corresponding to the formula:



40 13. A method of electrodepositing chromium upon a cathodic base which comprises passing an electrolytic current from an anode to said cathodic base through a chromium electroplating bath of a pH of about 7 consisting of an aqueous solution of a complex salt of trivalent chromium corresponding to the formula:



References Cited in the file of this patent

UNITED STATES PATENTS

1,777,121 Linick ----- Sept. 30, 1930

FOREIGN PATENTS

668,751 France ----- July 22, 1929